

## UNITED STATES PATENT OFFICE

JOHN P. WETHERILL, 3D, OF WASHINGTON, DISTRICT OF COLUMBIA, ASSIGNOR TO  
AMERICAN MAGNESIUM METALS CORPORATION, OF PITTSBURGH, PENNSYLVANIA,  
A CORPORATION OF DELAWARE

## MAGNESIUM ALLOY

No Drawing.

Application filed May 8, 1931. Serial No. 536,075.

This invention relates to improvements in alloys and more particularly to an improved magnesium base alloy.

As is known, there is a considerable demand in technical fields for alloys which combine the desirable properties of light weight and relatively high mechanical strength. Heretofore a number of magnesium alloys have been proposed to fulfill these requirements.

I have found that a very satisfactory alloy combining the desirable properties of lightness in weight, together with relatively high tensile strength and satisfactory resistance to corrosion, may be prepared by alloying minor amounts of cobalt with magnesium. The alloy may very simply be made up by adding small quantities of cobalt to molten magnesium maintained under a flux. The preferred form of flux may comprise a mixture of magnesium chloride, potassium chloride and sodium fluoride. Preferably the vessel in which the alloying is carried out is lined with magnesium oxide or some equivalent material so as to maintain the components of the final alloy in a relatively pure condition, and particularly to maintain it free from iron and especially from metals which are decidedly electro-negative to magnesium, such for example as copper.

The process has been actually carried out for the manufacture of an alloy in which a quantity of magnesium was fused in a vessel, and out of contact with iron, and to which cobalt in small amounts was added. In carrying out the process it is advisable to either add the cobalt in small amounts to the mass of molten magnesium or to provide some method of cooling in the event that the cobalt is added in relatively large quantities, since the reaction is quite exothermic and if too much heat is generated, burning of the magnesium occurs.

As a typical example of the method of manufacture and of the alloy a small quantity of cobalt was added to a quantity of magnesium which was substantially free from copper and iron. It was found that the components alloyed very readily. The operation was carried out in a vessel lined with

magnesium oxide and the molten magnesium was protected from the air with a flux constituted by a mixture of magnesium chloride, potassium chloride and sodium fluoride. The alloy was allowed to cool and a small sample was analyzed to determine particularly the foreign elements and the percentage of cobalt. The percentage of cobalt was determined by dissolving a piece in hydrochloric acid solution and then treating with nitro-beta-naphthol to precipitate the cobalt. It was found that the alloy contained approximately .5% of cobalt and was substantially free from copper and iron.

The hardness of the alloy of the above composition was determined by a Rockwell machine using a  $\frac{1}{8}$ " ball and a 100 kilogram load. Several tests of the hardness disclosed values varying from 82.8 to 87.4, and more specifically four readings disclosed the following hardness numbers: 82.8, 85.4, 87.5 and 87.4. The hardness of this alloy, it will be noted, compares very favorably with known commercial alloys. For example pure magnesium (99.9), extruded at 300° C., has a hardness of 46 (100 R, B  $\frac{1}{8}$ ), i. e. the hardness number of 46 using the Rockwell machine with a 100 kilogram weight and a  $\frac{1}{8}$ " ball. This sample of magnesium has a tensile strength of 28,650 lbs. per sq. in. A magnesium alloy of 3% manganese, 4% aluminum and the remainder magnesium, has a hardness of 42 (100 R, B  $\frac{1}{8}$ ). The particular alloy of this test was sand cast at 650° C. The above mentioned standard alloy, on being rolled and heat treated at 450° C. and quenched, had its hardness increased to 59.6 (100 R, B  $\frac{1}{8}$ ) and disclosed an increase in tensile strength. This same commercial alloy, namely the ternary magnesium aluminum manganese alloy, when extruded at 290° C. and rolled at 450° C., has its hardness increased to 70.1 (100 R, B  $\frac{1}{8}$ ).

It was found that additional amounts of cobalt, when alloyed with magnesium, likewise produced improved alloys. Thus, for example, cobalt may be added to magnesium to produce binary alloys having a fraction of a percent of cobalt up to approximately 5%. In making up alloys with these higher

percentages of cobalt care should be exercised in effectively cooling the mass, because as the cobalt percentage increases the exothermic heats of reaction increase to very near the burning point of magnesium.

It will be seen from a comparison of an alloy of the present invention with those of known commercial magnesium alloys that it is characterized by an exceptionally high 10 degree of hardness and even in the unworked condition has a higher degree of hardness than other commercial alloys.

It will also be observed that inasmuch as the alloy as made up is substantially free 15 from copper and contains as a secondary component an element which is relatively close to magnesium in the electro-chemical series, the tendency of the alloy to corrode due to galvanic action is relatively slight.

20 It is further found that the magnesium cobalt alloy is readily workable and machines very well. It is additionally characterized with a relatively high tensile strength. It will be understood, as recognized by those 25 skilled in the art, that the mechanical properties of the alloy may be improved within determinative or permissive limits by increasing the proportion of cobalt, and that similarly the mechanical properties may be 30 improved by working and heat treatment.

While a preferred embodiment of the invention has been described, it is to be understood that this is given merely by way of 35 example of the underlying principles of the invention. It is recognized that magnesium has been widely used as a deoxidizer in metallurgical operations and that proposals have been made to increase its efficiency as a deoxidizer by alloying it with very large portions of heavy metals for the purpose of 40 improving its characteristics for this purpose. These deoxidizers are in no proper sense commercial alloys. The present invention, therefore, is to be sharply distinguished from such 45 prior disclosures and relates to commercial alloys containing a relatively minor percentage of cobalt so as to produce an article which is characterized by a very low specific gravity as well as satisfactory mechanical properties.

50 I claim:  
1. A light weight alloy comprising from 90 to 99% of magnesium and the remainder cobalt.  
55 2. A light weight binary alloy comprising approximately 99% of magnesium and one percent of cobalt.

In testimony whereof I affix my signature.  
JOHN P. WETHERILL, 3d.